

# UNITED STATES PATENT OFFICE.

JACOB KINDLEBERGER, OF KALAMAZOO, MICHIGAN, ASSIGNOR TO THE KALAMAZOO  
VEGETABLE PARCHMENT CO., OF KALAMAZOO, MICHIGAN, A CORPORATION OF  
MICHIGAN.

## WATERPROOF PAPER AND PROCESS OF MANUFACTURE.

1,126,783.

Specification of Letters Patent.

Patented Feb. 2, 1915.

No Drawing.

Application filed February 15, 1912. Serial No. 677,802.

To all whom it may concern:

Be it known that I, JACOB KINDLEBERGER, a citizen of the United States, residing at Kalamazoo, Michigan, have invented certain new and useful Improvements in Waterproof Paper and Processes of Manufacture, of which the following is a specification.

This invention relates to improvements in waterproof paper and methods and process of manufacturing the same.

The objects of the invention are to provide a pliable waterproof sheet of paper of high strength and durability.

Objects relating to details and economies will definitely appear from the detailed description.

I accomplish the objects of my invention by the devices and means described in the following specification.

The invention is fully pointed out in the claims.

As the means which I make use of in carrying out my process are well known to paper manufacturers, I have not deemed it necessary to illustrate the same.

In carrying out my process, I take plain unglazed paper in the form of the waterleaf of any desired grade. The better the grade, however, the better the product and a pure cotton rag paper gives the best results. I subject the sheet of paper, by proper machines or devices, to the action of a solution of sulfuric acid of a test of about fifty-four degrees Baumé. The sheet is passed through this solution quickly, but is completely submerged and acted upon by the acid. The acid may safely test from fifty-three to sixty degrees. Any strength that will parchmentize and not burn the sheet is permissible. The sheet is then passed through a washer and thoroughly flooded and washed with clear water so that all the acid is flooded and washed away. The sheet is then thoroughly dried. The dried sheet is then subjected to the action of a solution of glycerin, the same being passed through a bath of glycerin, which is squeezed off by suitable rollers and the sheet dried by suitable fans, or otherwise, so that the water of the glycerin solution is practically dried away. That is to say, as much of the moisture is

evaporated as such drying means will eliminate. To secure best results, the glycerin treatment is repeated after about twenty-four hours. An antiseptic, such as carbolic acid, may be added to the glycerin. The solution of glycerin varies from sixty-five to seventy-five per cent. of glycerin, the balance being water. When the parchmentized sheet of paper has thus been treated to the glycerin bath, the same is rolled up into a tight roll and allowed to remain for a period of twenty-four hours or more. This insures that the glycerin shall permeate the parchmentized sheet as completely as it is possible for that to be accomplished by the glycerin, and the water has already been dried out of the same so far as that is practical. The glycerin solution can be varied in strength. It is desirable to incorporate the glycerin with the sheet in the minimum amount in practically a pure form to secure the best results. After the parchmentized roll of paper has been thus treated with glycerin for twenty-four hours or such a matter, the sheet is then passed through a paraffin coating machine and the hot paraffin is thoroughly forced into the sheet by the machine and will be found to permeate the same very effectively and completely waterproof the same. The result is that a very effectual waterproof sheet is secured, which is not liable to breakage from abrupt folding, and which is substantially as flexible as a sheet of cotton or linen fabric and is very strong and durable. The material thus produced is very desirable wherever any waterproof sheet is desired. It provides a substantially perfect waterproof bed covering, taking the place of a rubber sheet in all surgical cases, and is highly desirable for use in infants' beds, and as a diaper or for use with diapers. The same constitutes an effective waterproof wrapping for any article or purpose. The material being impervious to moisture and a non-conductor, can be wrapped over the top of a cake of ice in a refrigerator and prevent waste.

The process of applying glycerin and paraffin can be made use of in the treatment of ordinary parchmentized paper, but I prefer the exact method which I have indicated for the preparation of the parchment sheet

itself, as the best results follow and the glycerin and paraffin are more completely and effectively incorporated into the sheet in this way.

5 Having thus described my invention, what I claim as new and desire to secure by Letters Patent is:

1. The process of waterproofing paper, consisting in first subjecting a waterleaf sheet to the action of sulfuric acid fifty-four Baumé test; second, thoroughly washing the sheet and drying the same; third, subjecting the sheet repeatedly to a bath of from sixty-five to seventy-five per cent. of 10 glycerin solution; fourth, drying the sheet and rolling the same into a tight roll; fifth, then passing the parchmentized sheet thus treated with glycerin through a paraffin coating machine and forcing the paraffin 15 into the sheet, as described.

2. The process of treating paper consisting of first parchmentizing the sheet, second, cleansing and drying the same, third, impregnating the sheet with glycerin and 20 thoroughly incorporating the glycerin into 25

the same, and fourth, passing the said sheet through a paraffin coating machine and coating the same with paraffin, as described.

3. The process of treating paper, consisting of parchmentizing the sheet, impregnating the parchmentized sheet with glycerin and coating the said sheet with paraffin. 30

4. A waterproof sheet of paper suitably parchmentized by the sulfuric acid method and impregnated with glycerin and coated 35 and impregnated with paraffin, as specified.

5. A sheet of parchmentized paper impregnated with glycerin and carbolic acid and coated with paraffin.

6. A sheet of parchmentized paper impregnated with glycerin and an antiseptic and coated with paraffin. 40

In witness whereof, I have hereunto set my hand and seal in the presence of two witnesses.

JACOB KINDLEBERGER. [L. S.]

Witnesses:

M. PHINA WOODRUFF,  
MARGARET GLASGOW.